

## UNITED STATES PATENT OFFICE

1,976,745

## PAPER MANUFACTURE

Harold Robert Rafton, Andover, Mass., assignor  
to Raffold Process Corporation, a corporation  
of Massachusetts

No Drawing. Application December 6, 1932,  
Serial No. 646,025

19 Claims. (Cl. 92—21)

This invention relates to the manufacture of paper filled with alkaline filler.

The principal object of this invention is to produce paper substantially free from discoloration, which paper contains alkaline filler and fibrous material capable of discoloration by alkaline filler.

An important object is to produce substantially unsized paper filled with alkaline filler.

10 A further object is to produce substantially unsized paper filled with alkaline filler, the surface of which paper has a different pH value than the alkaline filler itself.

15 A further object is to produce substantially unsized paper filled with alkaline filler, the surface of which paper is substantially non-alkaline.

Other objects and advantages of my invention will become apparent during the course of the following description.

20 In my copending application Serial No. 501,674, filed December 11, 1930, now Patent 1,922,325, granted August 15, 1933 I disclose a method of manufacturing sized paper filled with alkaline filler by the application of size and size precipi-

25 tant to a paper web containing alkaline filler. Alternatively the precipitant may be applied to the paper mix and the size to the web, or the size to the paper mix and the precipitant to the web, or precipitated sizing may be applied to the

30 web.

In my copending application Serial No. 644,909, filed November 29, 1932, I disclose a method of manufacturing sized paper filled with alkaline filler wherein undeveloped, deteriorated or destroyed sizing is developed, or sizing is enhanced or preserved, by the application of a sizing affecting agent to a paper web containing alkaline filler.

The present invention deals with a method 40 similar to that employed in my last mentioned copending application, namely with the application to a fibrous web containing alkaline filler of an agent suitable for affecting the web in the desired manner. In the present invention, however, I am concerned with paper which contains material, particularly fibrous material, capable of being discolored by alkaline filler, and/or with substantially unsized paper.

In the manufacture of paper filled with alkaline filler, fibrous material may be used in certain cases which is not substantially all cellulose but which contains a portion and in some cases a considerable proportion of non-cellulosic material. This material when in contact with alkaline filler, especially at the temperature of the

paper machine drying cylinders, has in certain instances a tendency to become yellowish or brown or otherwise to change from the color it possesses when originally employed. An example of such a fibrous stock is what is known as "ground wood", which is a fibrous material obtained from wood by mechanical grinding processes, and which has ordinarily received no chemical treatment. There are other fibrous materials obtained by so-called semi-chemical processes, which contain a considerable portion of the non-cellulosic constituents of the cellulose-containing sources from which the fibrous materials have been derived, and such fibrous materials in certain cases are also subject to discoloration by the alkalinity of the alkaline filler under similar conditions. In other cases fibres which are known as chemical fibres, that is, which have been derived from the original cellulose-containing material by a relatively drastic chemical treatment which removes the major portion of the non-cellulosic content of the original cellulose-containing material employed, may contain residual portions of non-cellulosic material which may be subject to similar discoloration by alkaline filler. Or any of the classes of fibres mentioned above may have associated therewith certain residues or constituents derived from the various processes to which the fibre has been subjected, which when contacting with alkaline filler, especially on the driers, may cause a discoloration; or even in certain cases the cellulose constituent itself in contact with alkaline filler may cause a discoloration. Moreover, in certain cases in the manufacture of paper filled with alkaline filler certain coloring matters such as pigments or dyes may be employed which are attacked by alkaline filler, particularly at the temperature of the driers.

It is an object of the present invention substantially to prevent the discoloration in certain papers which may result from the reaction between alkaline filler and fibrous material or material associated with the fibrous material, or substantially to restore the original color in case such discoloration has taken place, also substantially to restore the color value of or substantially to prevent the deterioration of coloring matter affected by alkaline filler: all in the presence of alkaline filler.

In the manufacture of substantially unsized paper filled with alkaline filler, the paper produced is more or less alkaline in reaction, and it happens that in certain cases this alkaline reaction of the paper surface has an unfavorable

105

110

- effect on certain inks, colors and the like, and thus such papers at times are at a disadvantage compared with papers filled with non-alkaline filler. Thus, it will be apparent that the 5 production of a paper filled with alkaline filler having a surface reaction less alkaline than the alkaline filler with which it is filled, or even having a substantially non-alkaline surface reaction, that is one which is either neutral or in some 10 cases acid, will result in the obtaining of substantially improved results with such papers. It is an object of this invention to provide a method of manufacturing paper filled with alkaline filler, which paper possesses a surface reaction of a different pH value from its central portion, for example the surface reaction may be only mildly alkaline, that is, less alkaline than the alkaline filler from which it is made, or even in some cases substantially non-alkaline, i. e. either neutral or 15 acidic.
- 20 In the preferred practice of my invention I form a web containing fibrous material and alkaline filler, and to this web I apply a web affecting agent.
- 25 One illustrative example of the practice of my invention is as follows: I mix in a beater or other suitable mixing device alkaline filler and fibrous material susceptible of discoloration by alkaline filler, such as groundwood. There may also be 30 present in the furnish other fibrous material such as sulphite pulp or the like, which may if desired be substantially non-susceptible of discoloration by alkaline filler. The mix may also if desired contain other ingredients such as sizing agent, 35 or sizing agent and size precipitant. After giving the mix the proper preliminary preparation, it becomes ready for delivery to a web-forming device and when it is run off on such device a web containing alkaline filler is produced. To this 40 web I apply a web affecting agent and by this means the paper which would otherwise be discolored is either prevented from being substantially discolored or has its discoloration substantially discharged.
- 45 Another illustrative example, in this case one in which I substantially maintain in, or restore to, a web the desired color, in which web alkaline filler is present in association with a dye or pigment capable of being affected by alkaline filler, is as follows: I mix fibrous material and alkaline 50 filler in a beater or other suitable mixing device, together with a dye or pigment capable of being affected by alkaline filler. There may be present also if desired other ingredients such as sizing agent, or sizing agent and size precipitant. 55 I then subject the mix to the desired treatment, and run it off on a web-forming device to form a web which contains alkaline filler and the dye or pigment capable of being affected by alkaline 60 filler. To this web which would otherwise have the improper or deteriorated color value, I apply a web affecting agent whereupon the color of the dye or pigment is substantially maintained at, or restored to, its desired color value.
- 65 Another illustrative example of practicing my invention in the case where I desire to produce substantially unsized paper filled with alkaline filler, and where I desire to produce a paper having a less alkaline surface reaction than the paper 70 would have if it were not treated according to my invention, is as follows: I mix fibrous material and alkaline filler in the beater or other suitable mixing device, adding if desired an agent, preferably an acidic material such as alum, or size in 75 an amount insufficient to impart a substantial

degree of sizing to the resulting paper, and if desired a precipitant therefor. I then give the mix the desired treatment and run off the same on a web-forming device. There is thus formed a web containing alkaline filler, and to this web I apply a suitable web affecting agent, whereupon the paper produced will be found to have a less alkaline surface reaction than if the web affecting agent had not been applied.

80 In any of the above examples other paper-making ingredients may be added as desired such as starch and the like. It will also be understood that in any or all of these examples, the materials noted or other materials desired to be used therewith in the papermaking mix may be added in accordance with the minimizing principle, that is, under conditions favoring the minimizing of the time and/or intimacy of contact of the constituents of the mix, preferably at the dilute stage of the papermaking operation, as described in a 85 large number of my already issued patents. According to such principle one or more of the various papermaking ingredients such as acidic material as alum, alkaline filler, size, starch and the like may be added at the dilute stage of the paper- 90 making process.

95 It will be understood of course that the above examples are merely illustrative, and in no way limiting.

100 The web affecting agent which I employ for application to the web containing alkaline filler may be either gaseous, liquid or solid. Such web affecting agent must be of a nature which either reacts directly with alkaline filler or which compensates for or inhibits the action of alkaline filler 105 on the fibrous material, coloring matter or the like. For instance acidic material in general may function, such for example as acetic acid or other organic or mineral acid as sulphuric or phosphoric acid or acid salt such as sodium bisulphate. The 110 acids may conveniently be applied to the web in liquid form preferably in aqueous solution, but it is possible to apply at least certain of them such as formic, acetic, or hydrochloric acid in gaseous form; and also to apply acids or acid anhydrides 115 which occur in gaseous form at temperatures which will not substantially injure cellulose fibre. Thus, for example, carbon dioxide or sulphur dioxide may be employed although in such cases there should preferably be water or aqueous vapor 120 present in order to make them function properly.

125 Likewise the agent may be applied to the web in solid form for example as a solid acid, preferably finely powdered, such as solid organic acid, 130 or powdered solid salts such as sodium bisulphate or the like may be used. In this case also water should preferably be present in the web to affect the solution of the agent in order that it may have a proper effect on the web. Among other agents 135 which I may employ in addition to those mentioned are metallic compounds, preferably soluble, such for example as sodium bisulphate and the like, which may be non-acid, or which may be acid, such as aluminum sulphate (ordinary alum) 140 or other aluminum compound such as aluminum chloride or stannous chloride, lead acetate, and the like. In certain cases, for example where a discoloration having its origin in the fibrous material is present in the web or may be developed 145 therein, bleaching material may be employed, which may be either oxidizing in action, such as hypochlorites, or reducing such as bisulphites.

150 However in general, from the standpoint of economy and effectiveness, I prefer to use alum

as my web affecting agent and because of convenience of handling it, I prefer to apply it in aqueous solution.

The application, i. e. exposure, of the web affecting agent in gaseous or vapor form to the web may take place when the web is either in the wet or in the dry condition, but preferably when it is in the wet condition, and will ordinarily require a container, hood or the like in which the web affecting agent may be exposed to the web. This may suitably be provided by enclosing that part of the paper machine at which the exposure is to be made in a suitable hood or enclosure or the like, which may be at atmospheric pressure, superatmospheric pressure, or subatmospheric pressure such as in a vacuum of suitable degree, as best meets the particular case; or such agent may be applied to the web independently of the paper machine in a special applying device.

The application of a liquid to the web, and this is my preferred method, may conveniently take place on the paper machine but here again as in the case of the gaseous agent, the liquid may if desired be applied to the web as a process independent of the paper machine. The above statements relative to place of application of a liquid are equally pertinent to the application of a solid web affecting agent.

The application of the web affecting agent to the web may take place while the web is either in the wet or the substantially dry condition, but in my preferred practice of using a liquid agent such as alum solution, I prefer to apply it to the already formed wet web after it has left the web-forming device as this fits in most conveniently with the ordinary papermaking operation and does not usually require special driers subsequent to the point of application of the agent, as might be the case if the agent were applied to the dried or almost dry web. It will be understood, however, that where I speak of applying web affecting agent to the web, I mean to include in the definition of "web" and as within the scope of my invention not only the already formed wet or dry web, but also the web as it exists in its formative or forming state at any point on the web-forming device between the point of delivery of the mix to the web-forming device and the point of delivery of the formed web from the web-forming device; and of course it will be understood that such application may take place to either side of the web, that is, either to the top or the bottom or to both.

In order to affect the alkaline filler near the surface more than that at the center of the web, it is of course necessary to apply the web affecting agent to the surface or surfaces of the web, but in certain cases such for example as where I wish to prevent discoloration or decoloration by alkaline filler, it will of course be understood that while the web is on the web-forming device the application of the web affecting agent may in such instances include the case where the agent may be introduced at the surface, as well as the case where the agent may be introduced within the forming web by suitable introducing devices.

In the application of the web affecting agent in solution to the web, any known form of device for applying liquids to a paper web may be employed; for example the web may be passed through a trough or vat containing the solution, or the solution may be transferred to the web by brushes, for example rotary brushes, or by contact rolls, or by supply boxes or rolls on the press rolls or other rolls, or by spraying or the like. In the case of spraying, the spray may be rela-

tively coarse, or it may be very fine so as to be in the form of a mist, if desired. My preferred equipment is, however, arranged at the presses, preferably at the third press, or even better at the smooth rolls if the machine be equipped with such rolls. At such points, the web has lost most if not all the water which it will lose by pressure and is in a reasonably absorbent condition. Thus if the paper machine be equipped with a third press roll which may be operated preferably without felts, two applying rolls contacting directly with the two third press rolls may be used to apply the alum solution to the wet web. Of course it will be understood that the contact rolls are supplied with the alum solution by appropriate means such as immersion in supply boxes, troughs, or the like, or by contact with other rolls, carrying the alum solution, or other suitable means. Optionally, and in certain cases this is a desirable procedure, the alum may be applied by an applying roll which contacts directly with the web itself and as will be apparent either in this case or in the case of press roll application, the alum may be applied either to one or both sides but the application to both sides of the web is the more general procedure.

In certain cases the web affecting agent may be applied by means of the felt or felts normally contacting with the web on the paper machine, or even by means of small independent traveling felt or felts, or belts, contacting with the web. In such cases the agent may be applied previously to the felt or the like, or may be applied at the nip of the contacting web and felt. However, the application by roll or rolls is as simple as any and thoroughly practical, and hence is a very convenient one to use. In order to obtain more complete penetration of the web by the web affecting agent, the web may be led over a suction box, roll, or the like at or subsequent to the point where the web affecting agent is applied to the opposite side of the web, particularly in the case where the web affecting agent is applied only to one side of the web, or to the two sides at spaced intervals. If desired a felt, wire belt, or the like may be interposed between the suction device and the web to carry and/or support the web. In general the method of application in any given case is that which is best adapted for use at the particular point at which the agent is to be applied and should be chosen with regard to the particular conditions to be met in any given case, all of which will be apparent to one skilled in the art.

As the agent is preferably applied continuously to the web, suitable means for supplying it to the applying device, for example pumps, should be employed, and the amounts applied should preferably vary regularly with the paper machine speed and be adjustable to the various grades and weights of paper run.

After the application to the web of the web affecting agent, the paper may be dried in the customary manner if desired and calendered or otherwise finished according to the type of paper being made. The result of the application of this web affecting agent is, as the case may be, to produce a paper with a different surface reaction than would otherwise be produced, and/or to produce a paper in which alkaline filler and fibrous material and/or coloring matter susceptible to discoloration or decoloration by alkaline filler is present, in which the color is substantially preserved or restored. In certain cases also the ap-

80

85

90

95

100

105

110

115

120

125

130

135

140

145

150

lication of web affecting agent to the web reduces any tendency to stick at the press rolls, of course in such case the agent being applied before or at the press rolls; and also in certain cases if the agent is applied at the web-forming device a tendency in certain mixes toward foaming or filling up the dandy roll can be reduced.

It will be understood, of course, that my invention of restoring the color to, or preserving the color or in, a web containing alkaline filler and fibrous material capable of being deteriorated in color by alkaline filler, differs in principle from the practice of the prevention of discoloration of fibrous material by the impurities thereof, by acidification; as in my invention the co-presence of the discoloration and the alkaline filler responsible therefor prevents complete acidification of the admixture of the paper ingredients, such as is possible only when no alkaline filler is present, and it was hitherto believed to be impossible to prevent discoloration of fibrous material unless complete acidification or at least neutralization was effected.

While I do not limit myself to the concentration of alum solution to be applied, and it will be apparent that the concentration required will in any event be influenced by machine speed, type of paper manufactured, and other variables well known to one skilled in the art, nevertheless I can state that a 15 per cent. solution has been found to be satisfactory for my purpose, and this can be the one tried in practice first and then adjustment of the concentration may be made either one way or the other. However in certain cases, for example if suction is to be applied to the sheet to improve the penetration of the web affecting agent, a much more dilute solution may be employed for example 1 per cent. or thereabouts. Likewise the amount of alum to be applied is difficult to state definitely owing to the variation in conditions, and type of paper made, but it may vary in certain cases from a fraction of a per cent. on the total furnish up to several per cent., and this quantity may be conveniently controlled by the agent applying device in conjunction with the adjustment of the concentration of the solution applied.

It will be apparent that the application of the web affecting agent to the web, particularly if said agent be one which does not substantially react with alkaline filler, will merely result in the co-presence in the web of the agent and the alkaline filler, or such amount of the agent as is not used up, for example by its web affecting action, or otherwise. Of course such amount of agent will in general be concentrated more nearly at one or both surfaces than at the central portion of the web according as the application has taken place to one or both surfaces.

60 However, if the web-affecting agent be one which reacts with alkaline filler, such as an acidic reagent, such action will result in a change in the chemical composition of the alkaline filler, at least on the surface of the alkaline filler particles, the reaction taking place more particularly with those particles of the alkaline filler which are near the superficial part of the web, this action taking place either at one or both sides of the web according as the application of the agent is made to one or both sides of the web; and in certain cases as will be apparent the pH value of the compound formed will be different from that of the alkaline filler itself, in most cases less. For example, if acetic acid be used as the agent and calcium carbonate as the filler, a cer-

tain amount of calcium acetate may be produced. On the other hand if, with calcium carbonate, an acid or an acid salt be used of which the calcium salt is substantially insoluble, that corresponding salt will be formed. For example, if phosphoric acid or an acid phosphate be the agent used, calcium phosphate will be formed. If sulphuric acid or acid sulphate such as alum be used, calcium sulphate will be formed, as well as aluminum hydroxide or other aluminum compound where alum is used.

By the term "alkaline filler" I mean substantially water insoluble filler which when agitated in contact with freshly boiled distilled water, say for an hour, will impart a pH value to such water greater than 7.0, that is, which will be on the alkaline side of the neutral point. Among fillers in this group may be mentioned calcium carbonate, of which lime mud from the causticizing process is one form; calcium carbonate magnesium basic carbonate employed in the paper disclosed in my United States Patent No. 1,595,416, issued August 10, 1926; calcium carbonate magnesium hydroxide disclosed in my United States Patent No. 1,415,391, issued May 9, 1922, and other substantially water insoluble normal or basic carbonates of alkaline earth metals, (which expression is herein intended to include magnesium), or compounds, double salts, or other physically associated mixtures of these with one or more other acid soluble materials of a substantially water insoluble nature. By the term "alkaline filler" I also intend to include fibrous material and/or other material such as paper coating constituents or the like containing one or more compounds of the character referred to, such as "old papers" or similar papers, "broke", or the like.

When I use the word "paper" herein, I use it in the broad sense to include products of manufacture of all types and of all weights and thicknesses, which contain as an essential constituent a considerable amount of prepared fibre and which are capable of being produced on a Fourdrinier, cylinder, or other forming, felting, shaping or molding machine.

Cross reference is hereby made to my copending application Serial No. 672,901, filed May 25, 1933, having certain related subject matter, as well as to my copending application, of which said application is a division, namely application Serial No. 534,462, filed May 1, 1931, now matured into Patent No. 1,914,526, issued June 20, 1933.

While I have described in detail various embodiments and examples of my invention, it is to be understood that the details of procedure and equipment, the proportions of ingredients, and the arrangement of steps may be widely varied without departing from the spirit of my invention or the scope of the subjoined claims.

I claim:

1. Paper filled with alkaline filler including among its ingredients alkaline filler and coloring matter capable of deterioration by alkaline filler in the presence of moisture at the temperature of paper machine driers, said coloring matter being present in substantially undeteriorated condition.

2. Paper filled with alkaline filler including among its ingredients alkaline filler and fibrous material capable of discoloration by alkaline filler in the presence of moisture at the temperature of paper machine driers, said fibrous material being present in a condition substantially free from discoloration.

3. Paper filled with alkaline filler and contain-

80

85

90

95

100

105

110

115

120

125

130

135

140

145

150

- ing groundwood at least one surface of which paper has a different pH value than the central portion thereof. 4. Paper filled with alkaline filler and containing groundwood, at least one surface of which paper is less alkaline than said alkaline filler. 5. Paper filled with alkaline filler and containing groundwood, said paper being less alkaline at least one of its surfaces than it is in the central portion thereof. 6. Paper filled with alkaline filler and containing groundwood, at least one surface of which paper is substantially non-alkaline. 7. Substantially unsized paper filled with alkaline filler, at least one surface of which has a different pH value than the central portion thereof. 8. Substantially unsized paper filled with alkaline filler, at least one surface of which paper is less alkaline than said alkaline filler. 9. Substantially unsized paper filled with alkaline filler, said paper being less alkaline at at least one of its surfaces than it is in its central portion. 10. Substantially unsized paper filled with alkaline filler, at least one surface of which paper is substantially non-alkaline. 11. Substantially unsized paper filled with alkaline filler, at least one surface of which paper is acidic. 12. Substantially unsized paper filled with alkaline filler having a conversion product formed in situ from alkaline filler adjacent at least one of the surfaces of said paper. 13. Substantially unsized paper filled with alkaline filler, the particles of said filler near the surface of said paper having a coating thereon comprising a compound of a lower pH value than said alkaline filler, said compound having a higher concentration adjacent at least one of the surfaces of said paper than it has at the central portion of said paper. 14. Substantially unsized paper filled with alkaline filler, having a substantially non-alkaline compound formed in situ from alkaline filler adjacent at least one of the surfaces of said paper. 15. Substantially unsized paper filled with alkaline filler, the particles of said filler near the surface of said paper having a coating of substantially non-alkaline compound thereon, said non-alkaline compound having a higher concentration adjacent at least one of the surfaces of said paper than it has at the central portion of said paper. 16. Substantially unsized paper filled with alkaline filler comprising calcium carbonate at least part of which is superficially coated with a reaction product of a pH value different from said calcium carbonate, said reaction product being formed in situ. 17. Substantially unsized paper filled with alkaline filler comprising calcium carbonate at least part of which is superficially coated with calcium sulphate. 18. Substantially unsized paper filled with alkaline filler, containing residual substantially unaffected web affecting agent adjacent at least one of the surfaces of said paper. 19. That step in the manufacture of paper, which paper includes among its ingredients alkaline filler and fibrous material capable of discoloration by alkaline filler, comprising applying web affecting agent to a paper web including said alkaline filler and said fibrous material.

HAROLD ROBERT RAFTON.

40

115

45

120

50

125

55

130

60

135

65

140

70

145

75

150